

(No Model.)

A. ROBINSON.

METHOD OF AND APPARATUS FOR ELECTRIC SOLDERING.

No. 449,258.

Patented Mar. 31, 1891.



WITNESSES:

*Wm. Brown*  
*Tom Day*

INVENTOR

*Almon Robinson*

# UNITED STATES PATENT OFFICE.

ALMON ROBINSON, OF LEWISTON, MAINE.

## METHOD OF AND APPARATUS FOR ELECTRIC SOLDERING.

SPECIFICATION forming part of Letters Patent No. 449,258, dated March 31, 1891.

Application filed April 18, 1890. Serial No. 348,584. (No model.)

*To all whom it may concern:*

Be it known that I, ALMON ROBINSON, a citizen of the United States, residing at Lewiston, in the county of Androscoggin and State 5 of Maine, have invented certain new and useful Improvements in Electric Soldering, of which the following is a full, clear, and exact description, which will enable others skilled in the arts to which it appertains to use my 10 improved process and to make the apparatus necessary therefor.

The processes of electric soldering heretofore in use are either analogous to those used for electric welding, or else consist in using 15 in the same way that an ordinary soldering-copper is used a piece of metal which has been heated either directly or indirectly by the electric current.

The object of my invention is to provide a 20 process which shall be applicable under a greater variety of conditions than those above mentioned.

My invention consists, primarily, in melting a definite amount of solder by passing an 25 electric current through a circuit into which it has been inserted and thereafter applying the melted solder to the joint to be made.

My invention further consists in keeping the solder at the desired temperature through 30 out the operation by passing through it a current of regulated quantity.

My invention further consists in raising the metal to be soldered to the requisite temperature by the combined effect of the heat 35 transmitted through the melted solder, and of the heating caused by the electric current which is shunted through the metal itself.

My invention further comprises various 40 features of the apparatus used, which are hereinafter fully set forth.

In the single figure of the accompanying drawing, H is a handle of wood or other insulating substance through which pass two copper rods C C', which converge toward each 45 other until their points are separated by a capillary air-space a. To the other end of the rods C C' are attached (preferably by electric welding) flexible conductors F F. One of these conductors terminates in a binding-post 50 P, the other in a resistance-box R, where the current passes through the desired number of

resistances r r to the swinging arm A, from which it passes to the source of electricity whose opposite pole is connected to the binding-post P. This source of electricity may be a primary 55 or a secondary battery, a continuous or an alternating current dynamo, or an alternating converter, the only limiting condition being that the apparatus used shall furnish a manageable current of sufficient volume to 60 have the necessary heating-power. As the object of the resistance-box shown is merely to vary the amount of current flowing through the circuit, any other device for conveniently varying the resistance of the circuit, or for 65 varying the electro-motive force acting therein, or for introducing a counter electro-motive force, can be substituted therefor when the circumstances attending a particular application of my process make it desirable to 70 do so. Flexibility of the conductors F F' may be obtained either wholly or in part by the use of joints, and the conductors may be rigid throughout where the desired application will admit of their use. 75

For particular purposes the rods C C' may be curved in any way which renders their manipulation easier, and their adjacent ends should be coated with tin or with an alloy with which the solder used will readily unite 80 when melted.

I prefer in most cases to bring the conductors C C' so near each other that the melted solder is drawn up into the space between them and retained there by capillary attraction; but under some circumstances they can be separated to a greater distance, if desired. 85

In carrying out my process I close the circuit at the capillary air-space a with a piece of solder-wire or with any other piece of solder of convenient size and shape. I next send through the circuit a sufficient current to melt the solder, which then rises into the capillary space and spreads over the surface of the copper rods in the same way as over 95 an ordinary soldering-tool. The pieces of metal to be joined having been coated with a flux and placed in contact, the points of the conductors C C', with their adhering solder, are placed upon the joint or near it. As the 100 temperature of the solder is kept up by the current flowing through it, it imparts heat

very rapidly to the metal with which it comes in contact, and heat is also imparted to this metal by that part of the current which is shunted through it from one point to the other of the conductors C C'. These heating effects are for the most part independent of the position of the conductors C C', as regards the joint. They may rest upon both the pieces of metal to be joined, or upon one, and the current may flow parallel to the joint or across it. When the joint is sufficiently heated for the solder to flow over it, the conductors C C' are moved along and new solder is added as needed. The melting and the distribution of the solder can go on at once when more convenient by making a suitable increase in the current, which throughout the operation is kept within such limits that the solder is at all times hot enough to flow freely, while the heat at no time rises high enough to injure the solder or the metal to be joined.

As my process is widely applicable in the arts, its details are necessarily modified to suit particular applications, and I claim the right to use such minor variations in the process and apparatus as would naturally occur to a person skilled in the art of soldering if called upon to apply my process to any particular case.

Having now fully described my invention, what I claim, and desire to secure by Letters Patent, is—

1. The process of electric soldering, which consists in passing an electric current through the solder to be used, thereby melting the

solder solely or principally by the heating effect, which is proportional to its own ohmic resistance, and thereafter applying the melted solder to the joint to be made, all as set forth.

2. The process of electric soldering, which consists in melting the solder by placing two metallic conductors in contact with it, and thereby making it a part of an electric circuit, applying these conductors with their adhering solder to the metal to be joined, heating this metal by the combined effect of the melted solder and of the electric current, and regulating the heat throughout by varying the current, all as set forth.

3. In apparatus for electric soldering, a pair of metal rods whose points are held at a predetermined distance apart by an insulating-handle, in combination with each other and with a source of electricity which is capable of sending a heating-current through them when the circuit is completed by either solid or fluid solder between the points of the rods, all as set forth.

4. In apparatus for electric soldering, the combination, with a source of electricity, of a pair of metal rods whose points are separated by a capillary space of such dimensions that melted solder will rise into it, all as and for the purpose set forth.

Signed in presence of two witnesses on the 3d day of April, 1890.

ALMON ROBINSON.

Witnesses:

EZRA H. WHITE,  
FRED L. LEAVITT.